

146

Patented Mar. 28, 1939

2,152,406

## UNITED STATES PATENT OFFICE

2,152,406

## METHODS OF PICKLING METALS

Albert Jean Ducamp and Marie Emile Alfred  
Baule, Chaville, FranceNo Drawing. Application December 8, 1936, Se-  
rial No. 114,871. In France December 10,  
1935

10 Claims. (Cl. 148—8)

Br. 488,656  
148-8

The present invention relates to methods and compositions for pickling metals, that is to say removing superficial impurities, including oxides, from the surface of said metals.

5 In many industrial applications (such for instance as the application of fatty varnishes upon metals, welds, etc.) the known methods of pickling in an aqueous medium have many drawbacks: preliminary removal of grease, attack of 10 the metallic parts that are not oxidized, necessity of rinsing with water after the treatment and of drying very carefully so as to avoid a new oxidation of the surfaces that have been pickled, all this to finally come back to the necessary fat 15 medium for applying fatty varnishes or some welds.

It was already suggested to perform the pickling operation in a fatty medium by means of certain aliphatic acids or the like, such as stearic 20 acid, abietic acid, etc. These methods have proved unsatisfactory, especially when it is desired to free ferrous metals from the  $Fe_3O_4$  oxide. The action of these acids is not sufficiently strong 25 and the metallic soaps that are formed by the combination of these acids with the metallic oxides are little soluble in fatty bodies. They rapidly form an insulating layer upon the metallic surfaces which stops the pickling operation.

On the other hand, it is a known fact that, 30 with the pickling agents known up to the present time, the products of the combination of the metallic oxides remain in suspension or in solution in the pickling bath, thus modifying its composition, gradually reducing its efficiency and making it impossible to regenerate it after a cer- 35 tain time of use. It is then necessary to get rid of the whole of the bath, which is then useless, which constitutes a rather delicate problem in the case of large baths and involves heavy expenses, for instance for establishing a new bath.

40 The object of the present invention is to provide a pickling method and composition of matter which obviates these drawbacks.

According to the present invention, in order 45 to efficiently and economically pickle iron, copper, their alloys, and also other metals, we treat their surface by means of a liquid having, in addition to the chemical properties necessary for dissolving metallic oxides, that of constituting a medium which is miscible neither with the water 50 which necessarily accompanies the combination of these oxides with the acids, nor with the various waste products of this reaction, this medium being of relatively low density so that said water and said waste products spontaneously separate, 55 due to the difference in the specific weights, from the medium in which they are produced.

This automatic separation first permits a higher efficiency of the pickling liquid owing to the 60 liquid circulation that takes place along the sur-

face of the piece. On the other hand, it will be easier to maintain the pickling liquid to the desired composition. This results from the fact that the aqueous liquid resulting from this separation can be decanted without difficulty, and, as its volume is proportional to the consumption of active product, it will suffice, in order to regenerate the pickling liquid, to replace the decanted portion by a substantially equal volume of a suitable regenerating liquid, containing a suitable percentage of the consumed products.

It is thus possible to make use of a pickling bath, if not indefinitely, as least for a very long time.

We may even apply the method in a thorough- 15 ly continuous manner when it is desired to pickle pieces on an industrial scale, with a constant and regular output. In this case, according to the present invention, it will suffice to provide means for permanently evacuating the waste products 20 of the reaction from the lower part of the bath, whereas the corresponding amount of regenerating liquid is also fed in a permanent manner to the bath.

The pickling liquid necessary to the applica- 25 tion of the method thus defined may be given various compositions and it may be used either in the cold or in the hot state.

It is, for instance, possible to constitute this liquid of alcohols or of phenols or of saturated or unsaturated aliphatic acids or hydrocarbons or mixtures of the same, either in the presence of glycerides or not, and of one or several stronger acids capable of dissolving in these alcohols or these phenols, such as hydrochloric acid, acetic acid, phosphoric acid, formic acid, lactic acid, 35 oxalic acid, etc.

As alcohols, we may employ, either alone or in mixture, methyl, ethyl, amyl, butyl alcohols and their higher homologues, and also glycols and their etherified and esterified derivatives, these alcohols or glycols containing, or not, a small amount of trioxymethylene. We may also make use of industrial mixtures of alcohols.

As phenols, we may make use of hydroxybenzene, methylhydroxybenzenes, and their higher homologues.

As fatty acids, we may make use of undecylenic acid, oleic, stearic acids, and the like.

Under the action of this bath, the metallic oxides of the surface to be pickled combine with the strong acids, yielding metallic compounds in an aqueous medium which possess the property of separating spontaneously by difference of density of the fatty medium in which they are 55 formed.

It is easy, under these conditions, to separate the residues from the main part of the bath and to regenerate the latter by addition of a weight of active substances equal to the weight of these 60

substances which is present in combination in the part that is removed, the regenerating liquid thus utilized being of a composition and degree of acidity different from those of the initial liquid.

We found that good pickling action can be obtained by making use, preferably in the hot state, of a mixture of an alcohol, undecylenic acid, and one or several stronger acids capable of dissolving in an alcohol, such as hydrochloric, acetic or phosphoric acid, in such manner that the metallic oxides of the surface that is treated combine with said acids and give rise to the formation of metallic complex compounds soluble in oily matters, which dissolve in the excess of fatty acid and of alcohol, the latter belonging to the group including anhydrous ethyl alcohol, butanol, glycol and its derivatives: methyl-glycol, ethyl-glycol, poly-glycol, said acidified alcohols containing or not small amounts of trioxymethylene in the dissolved state. For instance, if it is desired to pickle, according to the invention, a steel sheet covered with  $Fe_3O_4$  oxide, either rusted or not, this sheet is immersed into a mixture containing: one part and a half of undecylenic acid, one part and a half of hydrochloric acid, and seven parts of butanol, by heating to a temperature of about 80° C., the proportions above indicated being given in volumes.

It suffices, after that, to wash with benzene  $C_6H_6$ , or a mixture of gasoline and anhydrous alcohol for instance, so as to remove the last traces of iron oxide which have taken the form of complex compounds soluble in oil. The metal sheet, after treatment, is perfectly capable of receiving a fatty varnish, either in the cold state, or in an oven, or of being protected or welded in any suitable manner in an anhydrous medium.

According to the invention, the proportions of undecylenic acid and of the other acids soluble in the alcohols may vary, same as those of the solvents.

If it is desired that the pickling mixture should attack only the oxides, without exerting any action on the metal proper, according to the invention, we dissolve in the hot state in said pickling mixture a small amount of trioxymethylene, for instance from 3 per thousand to 3 per cent, and the pieces to be pickled are heated only to a temperature of 60° C.

It may be assumed that, in the hot state, in the presence of an acid mixture according to the present invention, trioxymethylene produces esters which are attacked by the metallic oxides, with regeneration of the trioxymethylene and the formation of metallic salts, while of course the pure metal is not capable of attacking said esters.

We will now proceed to give some specific examples of mixtures according to the present invention.

We may for instance make use of an initial bath consisting of

|                                                 | Per cent |
|-------------------------------------------------|----------|
| Undecylenic acid                                | 10       |
| Anhydrous acetic acid                           | 5        |
| Hydrochloric acid in aqueous solution (22° Bé.) | 15       |
| Butanol                                         | 70       |

If an iron sheet covered with  $Fe_3O_4$  is immersed in this bath, small aqueous droplets are formed under the oxide stains and they drop to the bottom of the bath, driving along, together with them, the iron salts, and the waste products of the reaction.

At ordinary temperature, the pickling action

is finished after 5 or 6 hours. At a temperature of 65° C., the operation is finished after only 30 minutes.

If the metallic piece is allowed to stand in the bath after the oxides have disappeared, the attack on the metal is negligible.

After the operation, the aqueous liquid present at the bottom of the bath is removed, same as the residues driven along, and it is possible to regenerate the bath by replacing the part that has been removed by a substantially equal volume of the following composition:

|                   | Per cent |
|-------------------|----------|
| Undecylenic acid  | 15       |
| Acetic acid       | 10       |
| Hydrochloric acid | 65       |
| Butanol           | 10       |

The proportions of these components are, in fact, variable and can be determined in actual practice according to the amount of metal to be pickled, its degree of oxidation, and so on.

The losses due to evaporation, dripping, etc. can be compensated by adding the suitable amount of the initial product.

After pickling, the pieces are brushed under a stream of water, then neutralized by means of a suitable basic bath, such as lime water, sodium carbonate, etc.

A slight layer of fatty matter will remain on the surface of the pieces and will facilitate their preservation by protecting them against a new oxidation.

For the application of phosphatation or metalization, or other protecting coatings, it will be often necessary to remove the whole of the grease from the pieces through one of the known industrial methods.

Of course, it is possible, without departing from the principle of the present invention, to apply the pickling product above described in any other way than in the form of a bath, for instance for replacing sanding. By way of example, this product may be employed by atomizing, coating, or again, mixed with an inert powdery product, in the form of a paste which may adhere for the desired time on the surfaces to be pickled. In the latter case, regeneration of the product will not be possible, but the spontaneous separation of the products of the reaction will have for its effect to create a kind of local circulation in all points of the surface, which circulation increases the efficiency of the pickling acids.

What we claim is:

1. A method for removing superficial impurities from metals, which comprises contacting said metals with a liquid water-repellent pickling composition which is a non-solvent for pickling residues and has a lower specific gravity than water.

2. A method for removing superficial impurities from metals, which comprises contacting said metals with a bath of a liquid, water-repellent pickling composition which is a non-solvent for pickling residues and has a lower specific gravity than water, to precipitate water together with said pickling residues as a lower layer; withdrawing said lower layer; and regenerating the bath for further use.

3. A method for removing impurities from metal surfaces, which comprises subjecting the surfaces to the action of a water-repellent pickling composition including an acid selected from the group consisting of hydrochloric acid, acetic acid, phosphoric acid, formic acid, lactic acid and oxalic acid, a higher aliphatic acid and an alcohol which is substantially immiscible with water.

4. A water-repellent pickling composition which includes a pickling acid selected from the group consisting of hydrochloric acid, acetic acid, phosphoric acid, formic acid, lactic acid and oxalic acid, a higher aliphatic acid and a hydrocarbon having a free hydroxyl substituent, which is substantially immiscible with water.

5. A water-repellent pickling liquid which has a lower specific gravity than water and includes a pickling acid, selected from the group consisting of hydrochloric acid, acetic acid, phosphoric acid, formic acid, lactic acid and oxalic acid, a higher aliphatic acid and a liquid alcohol selected from the group consisting of butanol and its higher liquid homologues.

6. A water-repellent pickling composition including hydrochloric acid, undecylenic acid and butanol.

7. A water-repellent pickling composition which includes a pickling acid selected from the group consisting of hydrochloric acid, acetic acid, phosphoric acid, formic acid, lactic acid and oxalic acid, a higher aliphatic acid, an alcohol which is

substantially immiscible with water, and a small proportion of trioxymethylene.

8. A water-repellent pickling composition including about 1.5 parts by volume of undecylenic acid, 1.5 parts by volume of hydrochloric acid and 5 7 parts by volume of butanol.

9. A water-repellent pickling composition which includes a pickling acid selected from the group consisting of hydrochloric acid, acetic acid, phosphoric acid, formic acid, lactic acid and oxalic acid, a higher aliphatic acid and a liquid phenol substantially immiscible with water.

10. A method for removing impurities from metal surfaces, which comprises subjecting the surfaces to the action of a water-repellent pickling 15 composition including an acid pickling agent selected from the group consisting of hydrochloric acid, acetic acid, phosphoric acid, formic acid, lactic acid and oxalic acid, a higher aliphatic acid and a liquid phenol substantially immiscible with 20 water.

ALBERT JEAN DUCAMP.  
MARIE EMILE ALFRED BAULE.